

## UNITED STATES PATENT OFFICE

2,602,739

## SIZING COMPOSITIONS AND THEIR PREPARATION AND USE IN PAPER

Hareo Jacob Tadema, Amsterdam, Netherlands,  
assignor to Shell Development Company, San  
Francisco, Calif., a corporation of DelawareNo Drawing. Application July 28, 1947, Serial  
No. 764,241. In the Netherlands April 14, 1943Section 1, Public Law 690, August 8, 1946  
Patent expires April 14, 1963

9 Claims. (Cl. 92-21)

**1** This invention relates to the sizing of fibrous materials such as paper, cardboard, textile threads or fabrics, imitation leather, and the like. It deals with improved sizing compositions which may be applied during or after manufacture of articles of such types. It also deals with a new method of producing sizing compositions and with improved articles of manufacture which have been sized or made water-repellent with the new compositions of the invention.

A wide variety of compositions have been used for the sizing of fibrous materials of different types. Rosin or colophony, for example, is commonly employed for paper sizing but many other resins, waxes, bituminous or asphaltic materials, tars, etc. have been proposed for such use. The usual practice is to apply an aqueous solution or suspension of the sizing agent to the fibers to be sized and precipitate the size in the fibers by addition of a suitable precipitant. Thus, in the manufacture of paper or cardboard, suspensions of colophony saponified with alkali hydroxides or carbonates are added to the fibers in the beater or Holland machine and precipitated with paper maker's alum or the like.

It has now been found that more advantageous sizing compositions comprise aqueous emulsions containing controlled proportions of colophony with the predominantly cyclic extracts obtainable from mineral oils, particularly petroleum oils. For best results, it is desirable not only to regulate the proportion of colophony to cyclic extract in the mixture but also to control the character of the emulsion, particularly with respect to fineness of the dispersion.

According to the invention, improved sizing compositions are produced by emulsifying together with water 5 to about 30 parts by weight of colophony with 95 to 70 parts by weight of the chosen cyclic extract, preferably 10 to 20 parts of colophony with 90 to 80 parts of the extract, preferably using an aqueous solution of a base having a concentration of 5% to about 30% base by weight and containing from approximately half to about double the amount of base required for complete saponification of the colophony used. If proportions of colophony to aromatic extract outside the foregoing limits are used, difficulties are encountered in producing dispersions of the desired uniformity and stability, and there is a marked drop in the sizing quality of the product.

The cyclic extracts used in the new compositions of the invention are the products of predominantly aromatic and naphthenic nature ob-

tainable by extracting petroleum or related oils, including hydrogenation products of coal and the like, with solvents which are selective for non-paraffinic constituents. A wide variety of polar solvents may be used for the preparation of such extracts, liquid sulfur dioxide, phenol, cresylic acid, furfural, beta,beta-dichlorethyl ether, nitrobenzene, the sulfolanes and sulfolenes, and the like being typical examples of suitable solvents. 5 U. S. Patents Nos. 2,023,375, 2,357,344, 2,360,859 and 2,365,898, for instance, describe solvents which may be advantageously used. Combinations of solvents, as phenol with cresylic acid or liquid sulfur dioxide with benzene or toluene, for instance, are useful and the use of the so-called double solvent process employing mutually immiscible solvents, e. g. cresylic acid with propane, also gives suitable extracts. Methods of this type which may be used are described, for example, in U. S. Patents Nos. 2,029,190, 2,124,602 and 2,322,083. There are also advantages in reextracting the initial extract with an immiscible solvent to improve the selectivity of the extraction. Thus, extraction of Edeleanu extracts of lubricating oils with gasoline or the like has been found to improve the sizing properties of the compositions produced therefrom in accordance with the invention. Other extraction methods which may be used are described, for example, in U. S. Patents Nos. 2,081,721, 2,114,524 and 2,139,392. Extractive distillation may be used in place of or in combination with the previously mentioned extraction methods, suitable processes being described, for example, in U. S. Patents Nos. 2,109,157 and 2,407,820.

35 Extracts of heavier petroleum oils such as the lubricating oils and residual stocks are especially useful in the new sizing compositions of the invention, but other fractions of petroleum or related hydrocarbon products can also be used successfully as sources of the extracts. The extracts may be derived, for example, from lubricant distillates or bright oils or cylinder stocks which may, for instance, range in gravity from 15° to 8° API at 60° F. They may be obtained from any mixed type petroleum oil such as Mid-Continent or Coastal or California crudes or, in lower yields, from Pennsylvania type oils. For use in sizing in accordance with the invention, extracts boiling above 300° C. at 760 mm. Hg pressure are preferred, and most preferably extracts boiling from about 125° C. to 300° C. at 1 mm. Hg pressure are used. Extracts obtained from narrow fractions as described in U. S. Patent No. 2,115,960 40 may be advantageously employed. It is often

advantageous to fractionate the initial extract to separate fractions of especially advantageous properties; thus, for instance, it has been found that the higher boiling 50% to 75% of an Edeleanu extract of lubricating oil gives superior sizing judged by permeability to water of sized paper.

In order to obtain emulsions of the most desirable particle size it is advantageous to melt together the rosin and cyclic extract in the specified proportions and add the aqueous alkaline solution to the viscous mixture with suitable agitation. In this way a moderately fine, quite uniform, emulsion of the water-in-oil type is formed in which the average diameter of the particles, which are quite uniform in size, is of the order of about 10 microns or less. On further dilution of this initial emulsion with water the type of the emulsion is reversed and an extremely fine oil-in-water type emulsion is formed with particles of less than 1 micron, usually of the order of 0.1 micron, average diameter. The transition point for the change in the type of emulsion generally is at about 40% to about 50% water in the emulsion. No important difference in results has been observed when using rosins of different origins in this process.

A wide variety of different alkaline solutions may be used in preparing the emulsions. Hydroxides or carbonates of alkali metals or ammonia are particularly suitable; sodium or potassium or ammonium hydroxides are preferred hydroxides because of their relatively low cost. The corresponding, particularly the sodium and potassium, carbonates require higher temperatures and are thus somewhat less preferable. Bicarbonates may be successfully used as may also alkaline earth hydroxides such, for example, as calcium and magnesium hydroxides, etc. The best results have been obtained with potassium hydroxide solutions.

As previously pointed out, at least 5%, and more preferably at least 10%, by weight of rosin based on the total amount of rosin and extract used should be employed, and the quantity of alkali should be from about one-half to about twice that required for saponifying the resinic acids present in the colophony, the alkali being supplied in the form of an aqueous solution of about 5% to about 30% concentration, most preferably about 8% to 15% concentration. It is advantageous where highly stable emulsions are desirable to use not more than the equivalent amount of alkali for saponifying the rosin, most preferably about 90% to 100% of the equivalent amount.

The most favorable results are obtained when the melted mixture of colophony and extract is vigorously stirred during the addition of the caustic solution. Using a cylindrical mixer having a central paddle rotating between fixed paddle blades, the particle size of the emulsion was inversely proportional to the rate of stirring in the first stage of emulsification. The rate of stirring has little influence in the second emulsification stage, very good oil-in-water type emulsion being obtained in some cases on simply pouring the initial water-in-oil paste into water. The addition of the caustic in the first stage is preferably slow and gradual. The further dilution with water may be carried out relatively rapidly.

It is desirable to control the temperature of the mixture of extract and rosin during the saponification stage to within a few degrees of

the melting point of the mixture, preferably a temperature between the melting point and about 10° C. higher is used. If the temperature is too low the emulsification is unfavorably affected due to insufficient saponification of the rosin, while at too high temperatures poor emulsification results from the coalescence of initially formed emulsion drops. A starting temperature of about 50° C. to 65° C. is satisfactory, depending upon the particular rosin and extract used. The temperature may be allowed to fall to about 40° C. at completion of the alkali addition and then may be reduced further by subsequent dilution.

The initially formed water-in-oil type emulsion is particularly suitable for shipment and storage, and may be used with or without dilution for the gluing together of fibers of imitation leather. For the sizing of paper or cardboard it may be added directly to the fiber pulp in the Holland beater where it is diluted and converted to an oil-in-water type emulsion. The diluted emulsion is also preferable for treating textile threads and fabrics to make them water-repellent.

The initially formed water-in-oil type of emulsions are usually dark brown in color but dilution to produce the oil-in-water type converts them to emulsions which are yellowish green by incident light and reddish by transmitted light. Lighter colored sizes may be obtained by suitable decolorization of the extract before emulsification.

In contrast with sizes usually used in the manufacture of paper and cardboard which are generally used in the form of very dilute emulsions, e. g. of about 0.1% to 0.5% concentration, the products of the invention can be used in much more concentrated form. Thus, in the manufacture of paper and cardboard they may be employed as 20% to 50% emulsions of the oil-in-water type quite successfully, and when so used, hydration of the pulp is promoted making possible shorter times in the beaters, but lower concentrations can also be employed.

The new sizes of the invention may be used without any other change in the paper-making process. They may be precipitated on the fiber with aluminum sulfate or the like. A pH of about 4.5 to 6, depending on the type of pulp, is desirable during precipitation. If necessary, the pH may be controlled by adding dilute acid in the beater. About 25 grams of aluminum sulfate per kilogram of dry stuff in the beater gives satisfactory precipitation. Too much aluminum in the paper should be avoided as it adversely affects the permeability to water.

The emulsions of rosin and lubricating oil extract prepared according to the invention are highly stable. For instance, no flocculation was produced in a 0.04% emulsion with a particle size of 0.12 micron on addition of hydrogen chloride to 1/40 normal or of aluminum sulfate to 1/80 normal. The base in this emulsion had a normality of only 0.00013, so a hundred-fold excess of the acid or aluminum sulfate did not result in coagulation. However, in the presence of sulfite pulp a five-fold quantity of aluminum sulfate calculated on the base present was sufficient for complete precipitation. Although the emulsions do not readily coagulate, they occasionally show some phase separation on long standing but gentle shaking renders the emulsion immediately homogeneous again. Most stable emulsions are prepared at a pH below 9.5, preferably at about 8 to 9, and if the initial emulsion is too alkaline it can be given the desired pH by

adding a weak acid. Addition of small amounts of protective colloids, such as casein and gums, may be used to ensure the unlimited stability of the new emulsions.

Tests with kaolin and the like as fillers have shown that the sizes of the invention may be used with filled as well as unfilled papers. The new sizes also do not give any complications with paper dyestuffs. They are not only cheaper than the usual sizes but also have the advantage that the sizing effect obtained is greater than would be expected from sizing with either of the constituent parts of the product alone.

The following examples illustrate typical applications of the sizes of the invention and show their advantages in sizing paper of various kinds.

#### Example I

From a Kraft cellulose three papers were prepared, each having a weight of 100 g. per sq. m.

In the manufacture of the first paper sizing was carried out with an emulsion of an Edeleanu extract of lubricating oil, in the preparation of which a sodium soap of oil-soluble acids (obtained by treating a mineral lubricating oil with sulfuric acid) was used as emulsifier. This paper contained 0.9% by weight of Edeleanu extract calculated on dry paper substance.

A water-permeability test showed that the water had permeated the paper after 15 seconds.

In the manufacture of the second paper use was made of an emulsion of colophony wholly saponified with KOH. This paper contained 0.2% by weight of colophony, calculated on dry paper substance.

In the water-permeability test the water permeated the paper after 50 seconds.

In the manufacture of the third paper use was made of a size consisting of an emulsion prepared from a mixture of 80% by weight of the Edeleanu extract applied also for the first paper and 20% by weight of colophony, which mixture was entirely saponified with KOH of 10% concentration. This paper contained 1.0% by weight of the mixture, calculated on dry paper substance.

In the water-permeability test the water permeated the paper only after 125 seconds.

#### Example II

Twenty parts by weight of colophony were mixed, while heating, with 80 parts by weight of distillation residue of an extract prepared by treating a mineral lubricating oil with sulfuric acid. To obtain this residue the extract was distilled off to about one-half, while applying steam and vacuum.

Now to the colophony-residue mixture, having a ring and ball melting point of about 50° C., there was added so much of a 10% potassium hydroxide solution as to ensure the saponification of 90% of the colophony. The potassium hydroxide solution was slowly added to the mixture while intensively stirring. The temperature at which the saponification was effected amounted to 60° C.

A "water-in-oil" emulsion was obtained which, after being cooled to 40° C., was mixed while stirring with such an amount of water of normal temperature as to produce a 40% "oil-in-water" emulsion.

The emulsion thus obtained, in spite of its high concentration, was still thinly liquid and had a green color with incident light. The average particle size amounted to 68 millimicrons.

A Kraft-cellulose paper was manufactured,

with application of the above emulsion, on a Fourdrinier machine. This paper contained 1.0% by weight of the colophony-Edeleanu extract-residue mixture, calculated on dry paper substance. The sizing effect of this paper was excellent, the breaking strength, stretch, folding number and water resistance meeting all the standard specifications.

#### Example III

The advantages of using selected fractions of the initial lubricating oil extract are shown by the following results of comparative tests made with emulsions prepared as described in Example II. In each case bleached sulfite pulp was sized.

Using the entire Edeleanu extract of the lubricating oil, it was found that 2.75% by weight of size on the paper was required for normal sizing, i. e. 60 seconds permeability to water as measured by the ferric thiocyanate method in which the paper folded into a box is floated on an ammonium thiocyanate solution, the inside moistened with ferric chloride solution and the time measured for a red coloration to develop.

Extraction of the Edeleanu extract with gasoline before removal of the sulfur dioxide therefrom gave a concentrate in 65% yield after removal of solvents which required only 0.94% size on the paper for normal sizing.

The distillation residue of the same extract (the higher boiling 24%) required only 0.63% size for normal sizing. The 50%-75% fraction of the distillation required 1.50% for normal sizing and gave a very light colored size.

#### Example IV

In comparative tests of sizing Kraft pulp with emulsions prepared on the one hand from colophony alone and on the other hand from a mixture of 20 parts of colophony and 80 parts of the gasoline extract of an Edeleanu extract of lubricating oil using the emulsification method of Example II, the permeability of papers containing 3% size was as follows:

|                                    | Seconds: |
|------------------------------------|----------|
| Colophony size -----               | 156      |
| Edeleanu extract concentrate ----- | 182      |

It will thus be seen that the new sizing compositions of the invention offer many advantages, particularly with respect to economy of production and effectiveness of sizing compared with prior sizing compositions. While the invention has been described in considerable detail and several methods of applying it have been illustrated, it will be understood that other variations in its applications are feasible. Thus, for example, other sizing materials such, for instance, as are referred to in U. S. Patent No. 2,410,357, may be used along with the new sizes of the invention. Also, other acid-acting precipitating agents may be used instead of aluminum sulfate for sizing according to the invention. Still other variations are possible in the invention which is not intended to be limited to the specific procedures shown by way of example, nor by any theory proposed in explanation of the improved results which are obtained.

I claim as my invention:

1. A paper sizing composition consisting essentially of an aqueous emulsion having a pH of 8 to 9 of 10 to 20 parts of colophony saponified to the extent of about 90% to 100% and 90 to 80 parts of an Edeleanu extract of higher boiling

petroleum hydrocarbons wherein the particles have an average size of less than 1 micron.

2. An aqueous emulsion of the oil-in-water type suitable for sizing fibrous materials which comprises a stable dispersion in water of 5 to 30 parts by weight of substantially saponified colophony and 95 to 70 parts by weight of an extract of petroleum consisting largely of naphthenic and aromatic hydrocarbons, the water content of the mixture being at least 60% based upon the total weight of said dispersed components and water.

3. An emulsion of the water-in-oil type consisting essentially of water and a mixture of 10 to 20 parts by weight of colophony, at least half of which is saponified, and 90 to 80 parts by weight of a hydrocarbon mixture having a boiling point above 300° C. at normal pressure and consisting essentially of hydrocarbons extractable from petroleum with a solvent selective for aromatic hydrocarbons in the presence of paraffins.

4. A process of sizing Kraft paper pulp which comprises treating said pulp in a Holland machine with an aqueous emulsion formed by reacting a mixture of 10 to 20 parts by weight of colophony and 90 to 80 parts by weight of a raffinate from the extraction with gasoline of an Edeleanu extract of petroleum hydrocarbons boiling in the lubricating oil range with a 5% to 30% aqueous solution of at least one inorganic base selected from the group consisting of the hydroxides, carbonates, and bicarbonates of the alkali metals and of ammonia, and the hydroxides of calcium and magnesium, and adding to the mixture of pulp and oil-in-water type emulsion at a pH of 4.5 to 6 not more than 25 grams of aluminum sulfate per kilogram of dry stuff to precipitate said mixture on said fibers.

5. A process of sizing cellulose fibers which comprises intimately contacting an aqueous slurry of the fibers with an aqueous dispersion of a mixture of 5 to 30 parts by weight of colophony and 95 to 70 parts of an extract of petroleum consisting largely of naphthenic and aromatic hydrocarbons, which mixture has been emulsified with sufficient of an alkali solution of 5% to 30% concentration to saponify at least half of said colophony, and precipitating said dispersed mixture from an emulsion of the oil-in-water type onto said fibers with an acid-acting compound.

6. A paper product comprising cellulose fibers sized with a mixture of 10 to 20 parts of colophony by weight and 90 to 80 parts by weight of a raffinate from extraction with gasoline of an Edeleanu extract of lubricating oil.

7. Cellulose sized with a mixture of 10 to 20 parts by weight of colophony, at least half of which has been saponified with a potassium hydroxide solution of 8% to 15% concentration with 90 to 80 parts by weight of an extract obtained by extracting a petroleum oil fraction boiling between 125° C. and 300° C. at 1 mm. mer-

cury pressure with a polar solvent selective for aromatic hydrocarbons in the presence of paraffins.

8. Fibrous material having on its surface a mixture of colophony and aromatic and naphthenic hydrocarbons resulting from the precipitation with aluminum sulfate in the presence of said fibrous material of an emulsion formed by reacting a mixture of 5 to 30 parts of colophony and 95 to 70 parts by weight of an extract from extraction of a petroleum oil boiling in the lubricating oil range with a polar solvent having a selective solubility for aromatic and naphthenic hydrocarbons in the presence of paraffins with a 5% to 30% aqueous solution of an inorganic base selected from the group consisting of the hydroxides, carbonates, and bicarbonates of the alkali metals and of ammonia, and the hydroxides of calcium and magnesium, said base being present in an amount equivalent to from one-half to twice the requirement for saponification of the colophony.

9. In a process of sizing fibrous material by precipitating a sizing agent thereon, the improvement which comprises precipitating onto the fibers suspended particles of about 0.1 micron diameter from an emulsion of the oil-in-water type of 5 to 30 parts by weight of colophony and 95 to 70 parts by weight of the hydrocarbon extract of high boiling petroleum hydrocarbons, which extract is soluble in a solvent having a preferential solubility for aromatic hydrocarbons in the presence of paraffins, which emulsion contains at least 60% of water based upon the total weight of colophony, hydrocarbon extract and water and is formed by reacting said colophony and hydrocarbon extract with a 5% to 30% aqueous solution of an inorganic base selected from the group consisting of the hydroxides, carbonates, and bicarbonates of the alkali metals and of ammonia, and the hydroxides of calcium and magnesium.

HARCO JACOB TADEMA.

#### REFERENCES CITED

The following references are of record in the file of this patent:

#### UNITED STATES PATENTS

| Number    | Name           | Date           |
|-----------|----------------|----------------|
| 563,518   | Carmichael     | Sept. 29, 1896 |
| 1,806,474 | Lecocq         | May 19, 1931   |
| 1,833,038 | Pratt          | Nov. 24, 1931  |
| 1,943,975 | Lathrop et al. | Jan. 16, 1934  |
| 2,068,299 | Manson         | Jan. 19, 1937  |
| 2,117,256 | Rafton         | May 10, 1938   |
| 2,285,028 | Georgi et al.  | Jan. 2, 1942   |
| 2,301,298 | Light et al.   | Nov. 10, 1942  |
| 2,383,933 | Bump           | Sept. 4, 1945  |
| 2,415,408 | Bergier et al. | Feb. 11, 1947  |

#### OTHER REFERENCES

Chemical Abstracts, vol. 38, pages 863 and 864 (1944).